

March 27, 1934.

L. E. LEMAIGRE

1,952,810

ELECTRIC ARC CARBON

Filed Nov. 19, 1932

Fig. 1



Fig. 2



INVENTOR,

*Louis Edmond Lemaigre.*

*By*

*Stone, Boydon, Inack & Hahn.*

ATTORNEYS

## UNITED STATES PATENT OFFICE

1,952,810.

## ELECTRIC ARC CARBON

Louis Edmond Lemaigre, Paris, France, assignor  
to Compagnie Lorraine De Charbons Pour  
L'Electricite, Paris, France, a corporation of  
France

Application November 19, 1932, Serial No. 643,485  
In France December 4, 1931

6 Claims. (Cl. 176—134)

This invention relates to electric arc carbons for lighting purposes and more particularly to the carbons used in cinematograph projectors and the like.

Positive carbons of this kind generally consist of a shell of practically pure carbon and a core which comprises in addition to carbon, suitable mineralizing materials such as, for example, alkali or alkaline earth compounds, rare earth salts, etc. Generally, the carbon is tapered at one end so as to give it approximately the shape which it takes spontaneously in the course of combustion.

It has been found by experience that such carbons exhibit the following disadvantage. When a new carbon is compared with a carbon which has already been burnt, it is found that the chemical composition of the core is not the same in the end region, because the combustion has always deprived the hot end of the core of the most volatile mineral elements. The result is that the ignition of a new carbon always depends on thermal, chemical and electrical conditions which are variable and different in the course of use. One of the phenomena most frequently observed during this initial disturbed period consists in the appearance in the core of one or more holes, each of which corresponds to a zone of low luminosity and therefore gives rise to an irregular illumination of the cinematographic screen when the carbon is employed for picture projection.

The primary object of this invention is to overcome this disadvantage and this is achieved by slightly mineralizing the carbonaceous tip of the carbon by impregnation with a suitable metallic salt. Practical experience has shown that such impregnation, when correctly effected, remedies the disadvantage.

In order that the invention may be better understood, reference will be made to the following description taken in conjunction with the accompanying drawing in which Fig. 1 is a longitudinal sectional view illustrating diagrammatically a positive arc carbon as hitherto constituted; and Fig. 2 is also a longitudinal sectional view illustrating diagrammatically a similar carbon manufactured in accordance with this invention.

In Fig. 1, the carbon consists of a shell A of practically pure carbon and a core B which comprises, in addition to carbon, suitable mineralizing materials such as alkali or alkaline earth compounds, rare earth salts, etc. C is the tapered end ordinarily given to the unused carbon.

In Fig. 2 the carbon illustrated is similar to that in Fig. 1, except that a zone D situated at the tip

of the taper C has been impregnated with metallic salts, in accordance with this invention.

The impregnation of the zone D is effected by any well-known means, such as, for instance, by immersing the carbon tip in a suitable impregnating bath either at ordinary temperature or at an elevated temperature. It may be effected by placing the carbon with its tip in contact with a porous substance impregnated with a solution of the mineralizing metallic salt, this porous substance consisting, for instance, of asbestos paper, blotting paper, felt, or the like absorbent material. The impregnation may also be effected by dropping a regulated volume of the impregnating solution on the plane end of the tip C. For treating a number of carbon tips, a battery of nozzles may conveniently be provided under which pass the carbons, tips upwards. The solution penetrates into the mass of the carbonaceous shell by capillary action.

In order to illustrate the manner of carrying the invention into effect, the following example is given, but it is not to be regarded as limiting the invention to this precise method.

An electrode such as is represented in Fig. 2 consists of a shell A having a base of lampblack agglomerated and hardened by baking. The core B consists of a mixture of carbonaceous powder or graphite powder with an alkali salt, for instance, potassium silicate. The salt for impregnating the zone D of the tip C consists of potassium carbonate or borate and is made up into a solution containing 80 parts by weight of water and 20 parts by weight of the impregnating salt.

Some felt is soaked with this solution and the electrode is arranged upright on its tip with the latter in contact with the felt. Contact is maintained until the impregnating solution has penetrated the tip C to the desired depth D. If impregnation is effected in the cold, it has been found that periods of the order of 5 to 20 minutes are sufficient for this method of treatment for lampblack electrodes having an apparent density of about 1.45.

It is obvious that a similar method may be used, whatever the composition of the shell A (lampblack, retort carbon, petroleum coke, graphite, etc.) and also the mineralization of the core B, whether the latter comprises only alkali salts or other mineral materials such as, for instance, the alkaline earth fluorides, the fluorides or oxides of the rare earths, etc. The form of the tip C may also vary from a simple small chamfer to a point considerably tapered. The ratio of the diameter of the core to that of the shell may also

vary within wide limits such as, for instance, from 0.15 to 0.8, according to the purpose for which the electrode is to be employed. Further, the impregnating salts may be other than potassium carbonate and potassium borate, although the latter have been proved by experience to be the most suitable for use in the case of positive carbons for cinematographic purposes.

The depth of the zone D may be varied in accordance with the diameter and shape of the carbon and also with the electrical conditions under which it is to operate, but in all cases the zone of shell which is mineralized must not exceed that which is burnt away during approximately the first 2 to 5 minutes of operation.

I have observed what I believe to be the function and mechanism of action of such impregnation. It is known that the pure carbon arc is relatively resistant, whilst most of the metallic salts vaporized in the arc considerably increase its conductivity. The result is that on ignition, the arc is mainly fixed by the core since this alone comprises mineral elements. The current density to which this core is thus subjected may become very great and the vaporization of the mineral material take place with violence, so that the least break in the core, were it only visible under the microscope at the moment of ignition, becomes an active centre of vaporization and a hole soon forms at this same place. Once the excess of mineralizers is vaporized, a state of equilibrium is established and the combustion of the carbon progressively levels the edges of the hole, so that the latter has completely disappeared after several minutes ignition.

In cinemas, this disadvantage is so well-known that operators always take more care to "make the points" of their carbons by preliminary ignition for several minutes. However, with carbons treated according to the invention, the current density to which the core is subjected at the moment of ignition is limited because the mineral materials vaporized are drawn from both the core and the shell, so that holes are no longer formed, the regularity of operation is much more quickly established, such that the period necessary to "make points" is reduced under advantageous conditions for the user who thus obtains greater security and, at the same time, economy in carbons.

With reference to the foregoing explanation, it is to be understood that the invention is not to be regarded as being in any way limited thereby,

as obviously other explanations may be possible. It is sufficient to state that as a result of carefully conducted experiments with the invention, the improvements above-mentioned have been obtained.

The invention has been explained above with reference to positive arc carbons, but it must be clearly understood that in certain cases negative carbons having a slightly mineralized core can be subjected to the same process when perfect stability of operation is desired. Moreover, the invention can also be applied to the two-core carbons for operating on alternating current, but its application in this field is rather limited as the disadvantage remedied by the invention is much more rarely met.

I claim:

1. Electric arc carbon comprising a mineralized carbon core and a carbon shell surrounding said core, said shell being slightly mineralized at its operative end, while the remainder thereof consists of substantially pure carbon.

2. Electric arc carbon comprising a mineralized carbon core and a carbon shell surrounding said core, a small quantity of an alkali metal salt being dispersed throughout the operative end of said shell, while the remainder thereof consists of substantially pure carbon.

3. Electric arc carbon comprising a mineralized carbon core and a carbon shell surrounding said core, a small quantity of an alkali metal carbonate being dispersed throughout the operative end of said shell, while the remainder thereof consists of substantially pure carbon.

4. Electric arc carbon comprising a mineralized carbon core and a carbon shell surrounding said core, a small quantity of an alkali metal borate being dispersed throughout the operative end of said shell, while the remainder thereof consists of substantially pure carbon.

5. Positive arc carbon comprising a mineralized carbon core and a carbon shell surrounding said core, a small quantity of potassium carbonate being dispersed throughout the operative end of said shell, while the remainder thereof consists of substantially pure carbon.

6. Positive arc carbon comprising a mineralized carbon core and a carbon shell surrounding said core, a small quantity of potassium borate being dispersed throughout the operative end of said shell, while the remainder thereof consists of substantially pure carbon.

LOUIS EDMOND LEMAIGRE.